

## UNITED STATES PATENT OFFICE

2,367,468

## LUBRICANTS

Lawson W. Mixon and Clarence M. Loane, Hammond, Ind., assignors to Standard Oil Company, Chicago, Ill., a corporation of Indiana

No Drawing. Application August 15, 1942,  
Serial No. 454,975

13 Claims. (Cl. 252—48)

The present invention relates to lubricants, and particularly to improvements in lubricating oil compositions intended for use in internal combustion engines such as automobile and Diesel engines, under severe conditions, wherein corrosion due to acidity, piston ring sticking, cylinder wear, carbon sludge, varnish formation and viscosity increase may be encountered.

Straight petroleum lubricants are effective within certain defined limits of engine operating conditions but when these limits are exceeded, such lubricants frequently fail to give the desired performance demanded of them. Since in modern engines designed to give increased performance these limits are frequently exceeded, the use of straight mineral oils as lubricants produces undesirable conditions within the engine; thus varnish, carbon and sludge formation is excessive and corrosion of improved hard metal alloy bearings due to acidity is encountered.

It is an object of the present invention to provide a lubricant for internal combustion engines which will be effective in providing adequate lubrication for such engines. It is a further object of the invention to provide a lubricant which will not be inducive to the formation of varnish and/or sludge, nor inducive to an increase of viscosity. Another object of the invention is to provide a lubricant which will reduce engine wear and be non-corrosive to bearings. Other objects and advantages of the invention will become apparent as the description thereof proceeds.

We have discovered that the foregoing objects may be attained by employing a lubricating oil containing small amounts of the reaction product of a hydrocarbon or mixture thereof with chlorosulfonic acid. If desired, the reaction product may be neutralized by forming the metal salts thereof. Furthermore, the reaction product may be reacted with a sulfur and/or a phosphorus-containing compound, either before or after neutralization. Also, the hydrocarbon may be treated with the sulfur and/or phosphorus-containing compound before it is reacted with the chlorosulfonic acid.

The resulting compound will impart greatly improved characteristics to a lubricating oil when added in amounts of from about 0.05 per cent to about 10.0 per cent, and preferably in amounts of from about 0.5 per cent to about 3.0 per cent. The hydrocarbons used in the preparation of our improved compound should have a molecular weight of more than 160, and preferably of more than 500. Molecular weights of 800 or more are

particularly suitable. These hydrocarbons may be heavy oils, olefin polymers, paraffins, olefins, aromatics, alkylated aromatics, cyclic aliphatics, petroleum fractions, such as lubricating oil fractions, waxes, petrolatum, solvent extracts of petroleum fractions, cracked cycle stocks or condensation products of petroleum fractions, or the like. Aliphatic compounds are usually preferred over the aromatic compounds.

10     Essentially saturated hydrocarbons such as bright stock residuums, lubricating oil distillates, petrolatums, or paraffin waxes may be used. We may also employ the products resulting from the condensation of any of the foregoing hydrocarbons,

15     usually thru first halogenating the hydrocarbons, with aromatic hydrocarbons in the presence of anhydrous inorganic halides, such as aluminum chloride, zinc chloride, boron fluoride and the like.

20     We preferably employ olefin polymers having molecular weights above 160 and preferably between 500 and 3000. As olefinic starting materials for the production of such polymers, we may employ the individual olefins themselves,

25     mixtures of olefins, or mixtures of olefins and non-olefinic compounds. For example, the olefinic starting material may be propylene, butylene, amylanes, refinery gases containing normally gaseous olefins and cracked distillates or other 30     relatively low-boiling hydrocarbon mixtures containing normally liquid olefins and mixtures of normally liquid olefins, containing substantial amounts of dissolved normally gaseous olefins. We may also employ olefins obtained by the cracking of paraffin wax or by the dehalogenation of

35     alkyl halides, particularly long chain alkyl halides.

The polymers referred to above may be those obtained by polymerizing olefinic hydrocarbons in the presence of catalysts such as sulfuric acid, 40     phosphoric acid, or aluminum chloride, zinc chloride, boron fluoride and other catalysts of the Friedel-Crafts type. For example, we may employ the polymers resulting from the treatment of monoolefins preferably isomonoolefins such as 45     isobutylene and isoamylene and/or the copolymers obtained by the polymerization of hydrocarbon mixtures containing low molecular weight isolefins and normal olefins, preferably those of less than six carbon atoms.

50     We may also employ as the starting material the polymer or synthetic lubricating oil obtained by polymerizing unsaturated hydrocarbons resulting from the vapor phase cracking of paraffin waxes in the presence of aluminum chloride which 55     is fully described in United States Patents Nos.

1,995,260, 1,970,002 and 2,091,398. Still another type of olefin polymer which may be employed is the polymer resulting from the treatment of vapor phase cracked gasoline and/or gasoline fractions with sulfuric acid or solid absorbents such as fuller's earth whereby unsaturated polymerized hydrocarbons are removed.

Any of the above-mentioned hydrocarbons may be reacted with chlorosulfonic acid to produce a useful lubricating oil addition agent. However, it has been found that a greater improvement in the characteristics of the lubricating oil is attainable when the hydrocarbon-chlorosulfonic acid reaction product is neutralized with basic compounds such as the hydroxides, oxides, carbonates or bicarbonates of a metal, to form the corresponding metal salt of the reaction products. The metal salts may be the Na, K, Li, Ba, Sr, Ti, Ca, Co, Sn, Al, Zn, Cr, Fe, etc., derivatives of the reaction product. Other basic reagents may be used such as, for example, ammonia, or alkyl or aryl substituted ammonia such as amines.

The hydrocarbon-chlorosulfonic acid reaction product may be treated with a sulfur and/or phosphorus-containing compound such as S<sub>2</sub>Cl<sub>2</sub>, SCl<sub>2</sub>, P<sub>2</sub>S<sub>5</sub>, P<sub>2</sub>S<sub>3</sub>, P<sub>4</sub>S<sub>3</sub>, P<sub>4</sub>S<sub>7</sub>, PCl<sub>3</sub>, PCl<sub>5</sub>, P<sub>2</sub>O<sub>5</sub>, and the like. However, it is equally possible to react the hydrocarbon with such compounds before treating the hydrocarbon with the chlorosulfonic acid. When treating with the sulfur-containing and/or phosphorus-containing compound, a suitable catalyst such as sulfur or a Friedel-Crafts catalyst may be used, if desired. The metal salt of the hydrocarbon-chlorosulfonic acid reaction product may be treated with S<sub>2</sub>Cl<sub>2</sub>, SCl<sub>2</sub>, PCl<sub>3</sub>, PCl<sub>5</sub> and the like, if desired.

The reaction of the hydrocarbon or the sulfurized and/or phosphorized hydrocarbon with the chlorosulfonic acid may be carried out at temperatures of from about -40° F. to about 150° F. by merely adding from about 5% to about 50%, preferably about 10%-25%, by weight of the chlorosulfonic acid to the hydrocarbon or sulfurized and/or phosphorized hydrocarbon, and stirring the mixture from a few minutes to several hours. The reaction may be carried out in solvents characterized by being substantially non-reactive with chlorosulfonic acids. Typical solvents are cyclohexane, light normal hydrocarbons, chlorinated hydrocarbons and the like.

The chlorosulfonic acid reaction product, whether previously treated with the sulfurized

desired, subsequent to the neutralization step by treating with S<sub>2</sub>Cl<sub>2</sub>, PCl<sub>3</sub>, or the like.

The desired product, whether the hydrocarbon chlorosulfonic acid reaction product, the metal salt of the reaction product or the neutralized reaction product, may be used in lubricating oils, alone or in combination with other well-known lubricant additives, in amounts from about 0.05 per cent to about 10 per cent. Usually an amount of from 0.1 per cent to about 3 per cent gives highly favorable results.

As specific embodiments of our invention, the following examples are given by way of illustration and are not intended as a limitation of the invention.

#### EXAMPLE I

An isobutylene polymer having a Saybolt viscosity at 210° F. of 1200 sec. was treated with excess of ClSO<sub>3</sub>H with stirring at room temperature. The product was stirred with excess alcoholic KOH until the color (reddish-purple) had disappeared. The neutralized product was extracted with hexane and the hexane removed on the steam bath.

#### EXAMPLE II

A portion of the product from Example I, before neutralization, was treated with excess S<sub>2</sub>Cl<sub>2</sub> and warmed on the steam bath to remove unreacted S<sub>2</sub>Cl<sub>2</sub>. The product was then neutralized as in Example I.

The effect of small amounts of the above products on lubricating oils is determined by heating 250 cc. of the oil containing the desired amount of the addition agent at 330° F.-332° F. in a 500 cc. glass beaker in the presence of 5 square inches of copper and 10 square inches of iron. Four glass rods of 6 mm. diameter are suspended in the oil which is stirred at about 1300 R. P. M. with a glass stirrer having a 40 degree blade pitch. At stated intervals, oil samples are taken and sludge, acidity and viscosity values determined. The glass rods are also inspected for evidence of varnish formation thereon. Varnish values are based on a visual rating in which a glass rod free of any varnish is given a rating of 10, while a badly coated rod is given a rating of 1. Rods having appearances between these extremes are given intermediate values. The following data were obtained in the above described test:

Table

| Oil                                    | Vis.↑ in<br>crease<br>48 hrs. | Sludge (mg./10 g. oil) |         |         | Acidity (mg. KOH/g.<br>oil) |         |         | Varnish rating <sup>1</sup> |         |         |
|----------------------------------------|-------------------------------|------------------------|---------|---------|-----------------------------|---------|---------|-----------------------------|---------|---------|
|                                        |                               | 24 hrs.                | 48 hrs. | 72 hrs. | 24 hrs.                     | 48 hrs. | 72 hrs. | 24 hrs.                     | 48 hrs. | 72 hrs. |
| 1 Control oil                          | 1,158                         | 350                    | 975     | —       | 9.9                         | 16.6    | —       | 4-5                         | 1       | —       |
| 2 Control oil+1% product of Example I  | 285                           | 9                      | 103     | 377     | 1.9                         | 5.4     | 7.9     | 10                          | 9       | 6       |
| 3 Control oil+1% product of Example II | 298                           | 48                     | 171     | 379     | 2.3                         | 5.5     | 11.2    | 10                          | 10      | 10      |

<sup>1</sup> Saybolt Universal viscosity at 100° F. <sup>2</sup> Rating scale 10=no deposit, 1=very heavy deposit.

and phosphorized compound or not, may be neutralized by merely stirring with an excess of a metal hydroxide such as KOH, a metal oxide or a metal carbonate in water or alcoholic solution at approximately room temperature. If desired, a solid neutralization agent can be used at more elevated temperatures within the approximate range of from 100° F. to 400° F.

If the neutralized product has not already been treated with the sulfurizing and/or phosphorizing agent, this step may be carried out, if

65

The above data show the superiority of Examples I and II over the high grade control oil.

While we have described the use of our additives in lubricating oils, our invention is not limited to such use, since these reaction products may be employed in other petroleum products such as white oils, greases, waxes and the like, to increase the resistance thereof to oxidation and sludging, to inhibit the tendency thereof to corrode metals, and to deactivate metal surfaces which the above products may contact.

75

While we have described our invention with reference to particular embodiments thereof, other modifications may be made without departing from the scope and spirit of the invention. We do not wish to limit our invention to the examples set forth except in so far as the same is defined by the following claims.

We claim:

1. A lubricant comprising a lubricating oil normally susceptible to the formation of carbon, sludge, or varnish during use and an amount sufficient to reduce such formation of a product of the type obtained by the process comprising reacting a hydrocarbon in separate steps with chlorosulfonic acid and at least one agent selected from the group consisting of a sulfurizing agent, a phosphorizing agent, and a sulfurizing and phosphorizing agent and treating with a neutralizing agent subsequent to the reaction step with the chlorosulfonic acid. 10
2. A lubricant as claimed in claim 1 wherein the hydrocarbon is an olefin polymer. 15
3. A lubricant comprising a lubricating oil and from about 0.05% to about 10.0% of a product of the type obtained by the process comprising reacting a hydrocarbon in separate steps with chlorosulfonic acid, and at least one agent selected from the group consisting of a sulfurizing agent, a phosphorizing agent, and a sulfurizing and phosphorizing agent and treating with a neutralizing agent subsequent to the reaction step with the chlorosulfonic acid. 25
4. A lubricant comprising a lubricating oil normally susceptible to the formation of carbon, sludge or varnish during use and an amount sufficient to reduce such formation of a product of the type obtained by the process comprising reacting a hydrocarbon in separate steps with chlorosulfonic acid and a sulfurizing agent, and treating with a neutralizing agent subsequent to the reaction step with the chlorosulfonic acid. 30
5. A lubricant comprising a lubricating oil normally susceptible to the formation of carbon, sludge or varnish during use and an amount sufficient to reduce such formation of a product of the type obtained by the process comprising reacting a hydrocarbon in separate steps with chlorosulfonic acid and a phosphorizing agent, and treating with a neutralizing agent subsequent to the reaction step with the chlorosulfonic acid. 35
6. A lubricant comprising a lubricating oil normally susceptible to the formation of carbon, sludge or varnish during use and an amount sufficient to reduce such formation of a product of the type obtained by the process comprising reacting a hydrocarbon in separate steps with chlorosulfonic acid, a sulfurizing agent and a phosphorizing agent, and treating with a neutralizing agent subsequent to the reaction step with the chlorosulfonic acid. 40
7. A lubricant comprising a lubricating oil normally susceptible to the formation of carbon, sludge or varnish during use and an amount sufficient to reduce such formation of a product of the type obtained by the process comprising reacting a hydrocarbon in separate steps with chlorosulfonic acid and a sulfurizing and phosphorizing agent, and treating with a neutralizing agent subsequent to the reaction step with the chlorosulfonic acid. 5
8. A lubricant comprising a lubricating oil normally susceptible to the formation of carbon, sludge or varnish during use and an amount sufficient to reduce such formation of a product of the type obtained by the process comprising reacting a hydrocarbon in separate steps with chlorosulfonic acid and a sulfurizing agent and treating the product with a neutralizing agent. 15
9. A lubricant comprising a lubricating oil normally susceptible to the formation of carbon, sludge or varnish during use and an amount sufficient to reduce such formation of a product of the type obtained by the process comprising reacting a hydrocarbon in separate steps with chlorosulfonic acid and a phosphorizing agent, and treating the product with a neutralizing agent. 20
10. A lubricant comprising a lubricating oil normally susceptible to the formation of carbon, sludge or varnish during use and an amount sufficient to reduce such formation of a product of the type obtained by the process comprising reacting a hydrocarbon in separate steps with chlorosulfonic acid, a sulfurizing agent and a phosphorizing agent, and treating the product with a neutralizing agent. 30
11. A lubricant comprising a lubricating oil normally susceptible to the formation of carbon, sludge or varnish during use and an amount sufficient to reduce such formation of a product of the type obtained by the process comprising reacting a hydrocarbon in separate steps with chlorosulfonic acid, a sulfurizing and phosphorizing agent, and treating the product with a neutralizing agent. 45
12. A lubricant comprising a lubricating oil and from about 0.05% to about 10.0% of a product of the type obtained by the process comprising reacting a hydrocarbon in separate steps with chlorosulfonic acid and a sulfurizing agent and treating with a neutralizing agent subsequent to the reaction step with the chlorosulfonic acid. 50
13. A lubricant comprising a lubricating oil and from about 0.05% to about 10.0% of a product of the type obtained by the process comprising reacting a hydrocarbon in separate steps with chlorosulfonic acid and a phosphorizing agent, and treating with a neutralizing agent subsequent to the reaction step with the chlorosulfonic acid. 55

LAWSON W. MIXON.  
CLARENCE M. LOANE.